

# United States Patent Office

3,000,799

Patented Sept. 19, 1961

1

3,000,799

## NICKEL PLATING SOLUTIONS

Jack L. Towle, Cleveland, Ohio, assignor to The Harshaw Chemical Company, Cleveland, Ohio, a corporation of Ohio  
No Drawing. Filed Feb. 10, 1960, Ser. No. 7,783  
12 Claims. (Cl. 204—49)

This invention, which is a continuation-in-part of co-pending application Serial No. 833,398, filed August 13, 1959 now abandoned, which is a continuation-in-part of copending application Serial No. 796,211, filed March 2, 1959 now abandoned, relates to electrodeposition of bright nickel, that is, to the production of bright deposits of nickel which are bright as taken from the electroplating solution without buffing or polishing of any kind, and to the composition of solutions suitable for the production of such deposits.

Various solutions are known which are capable of producing bright nickel deposits. Some of these are of commercial value. Some are superior in particular respects while being inferior in other respects. Brightness, resistance to corrosion, long periods of trouble-free operation, adherence, ductility, freedom from pits, streaks and other irregularities, resistance to impurities in the bath are some of the factors which the art seeks to find in high degree and as many as possible in one process.

I have now discovered a group of closely related classes of compounds comprised within the general formula below which are excellent additives for use in acid nickel plating when used in connection with the aromatic sulfonates, sulfonamides and sulfimides. The latter may be referred to as control agents, the former as brighteners or auxiliary brighteners.

The brighteners with which the invention is concerned are those having the formula



wherein  $n$  is an integer from 1 to 6,  $n'$  is an integer from 1 to 6, R is a member selected from the group consisting of



where  $m$  is an integer from 1 to 6,



where  $R''$  and  $R'''$  are independently selected from the group consisting of hydrocarbon radicals and hydrogen; R' is a member selected from the group consisting of



where  $m$  is an integer from 1 to 6;



2



where  $R''$  and  $R'''$  are independently selected from the group consisting of hydrocarbon radicals and hydrogen; W is a hydrocarbon radical; X is an acidic radical selected from the group consisting of sulfate, sulfonate, halide and perchlorate radicals and  $t$  is an integer from 0 to 1 inclusive.

The classes of brighteners referred to are as follows:



where  $n$  is 2 and the hydrogen atoms may be substituted by methyl and where W is a hydrocarbon radical, X is an acidic radical selected from the group consisting of sulfate, sulfonate, halide and perchlorate radicals and  $t$  is an integer from 0 to 1 inclusive.



where R is a hydrocarbon radical having from 1 to 4 carbon atoms,  $n$  is 2 and the hydrogen atoms may be substituted by methyl, and where W is a hydrocarbon radical, X is an acidic radical selected from the group consisting of sulfate, sulfonate, halide and perchlorate radicals, and  $t$  is an integer from 0 to 1 inclusive.



where  $n$  is 2, and where W is a hydrocarbon radical, X is an acidic radical selected from the group consisting of sulfate, sulfonate, halide and perchlorate radicals, and  $t$  is an integer from 0 to 1 inclusive.



where R and R' are members independently selected from the group consisting of H and  $\text{CH}_3$ ,  $n$  is an integer from 1 to 3, and  $m$  is an integer from 1 to 2, and where W is a hydrocarbon radical, X is an acidic radical selected from the group consisting of sulfate, sulfonate, halide and perchlorate radicals, and  $t$  is an integer from 0 to 1 inclusive.



where  $n$  is an integer from 1 to 3 and  $m$  is an integer from 1 to 3, and where W is a hydrocarbon radical, X is an acidic radical selected from the group consisting of sulfate, sulfonate, halide and perchlorate radicals, and  $t$  is an integer from 0 to 1 inclusive.



where R is a hydrocarbon radical having from 1 to 6 carbon atoms, and  $n$  is 2, and where W is a hydrocarbon radical, X is an acidic radical selected from the group

consisting of sulfate, sulfonate, halide and perchlorate radicals, and  $t$  is an integer from 0 to 1 inclusive.

(7)



where  $n$  is 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(8)



where  $R$  is a hydrocarbon radical having from 1 to 6 carbon atoms and  $n$  is an integer from 1 to 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(9)



where  $R$  is a hydrocarbon radical having from 1 to 6 carbon atoms and  $n$  is an integer from 1 to 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(10)



where  $n$  is an integer from 1 to 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(11)



where  $n$  is an integer from 1 to 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(12)



where  $n$  is an integer from 1 to 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(13)



20

where  $R$  is a hydrocarbon radical having from 1 to 12 carbon atoms and  $n$  is 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(14)



30

where  $n$  is 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

35



40

where  $R$  is a hydrocarbon radical having from 1 to 6 carbon atoms and  $n$  is 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

45



50

where  $n$  is 2, and where  $W$  is a hydrocarbon radical,  $X$  is an acidic radical selected from the group consisting of sulfate, sulfonate, halide and perchlorate radicals, and  $t$  is an integer from 0 to 1 inclusive.

(17)



55

where  $W$  is a hydrocarbon radical,  $X$  is an acidic radical selected from the group consisting of sulfate, sulfonate, halide and perchlorate, and  $t$  is an integer from 0 to 1 inclusive.

(18)

The foregoing brighteners may be employed in the bright acid nickel plating solution at the rate of 0.0025 to 0.075 gram per liter.

Specific examples of brightener compositions according to the invention are set forth in Table I below.

TABLE I

| No. | Structure | Name                                                                                    | Preferred Concentration, Grams per Liter |
|-----|-----------|-----------------------------------------------------------------------------------------|------------------------------------------|
| 1   |           | 1, 5-Bis(2'-benzimidazolyl)-3-thiapentane, or Bis[B-(2'-benzimidazolyl) ethyl] sulfide. | 0.01-0.015                               |

Table I—Continued

| No.       | Structure                                                                                                                                                                         | Name                                                                                                      | Preferred Concentration, Grams per Liter |
|-----------|-----------------------------------------------------------------------------------------------------------------------------------------------------------------------------------|-----------------------------------------------------------------------------------------------------------|------------------------------------------|
| 2.....    | $\text{H}_2\text{N}-\overset{\text{O}}{\text{C}}-\text{CH}_2-\text{CH}_2-\text{S}-\text{CH}_2-\overset{\text{O}}{\text{C}}-\text{NH}_2$                                           | $\text{B},\text{B}'\text{-Thiodipropionamide, or Bis(2-carboxyamidoethyl) sulfide.}$                      | 0.0075-0.014                             |
| 3.....    | $\text{HOCH}_2\text{CH}_2-\text{S}-\text{CH}_2\text{CH}_2\text{OH}$                                                                                                               | $\text{Bis(2-hydroxyethyl) sulfide.}$                                                                     | 0.01-0.05                                |
| 4.....    | $\text{CH}_3\text{OCH}_2\text{CH}_2-\text{S}-\text{CH}_2\text{CH}_2\text{OCH}_3$                                                                                                  | $\text{Bis(2-methoxyethyl) sulfide.}$                                                                     | 0.01-0.03                                |
| 5(a)..... | $\text{HOCH}_2\text{CH}_2-\text{S}-\overset{\text{CH}_3}{\text{C}}=\text{HCH}_2-\overset{\text{O}}{\text{C}}-\text{H}$                                                            | 2-Formylisopropyl-2'-hydroxyethyl sulfide.                                                                | 0.005-0.01                               |
| (b).....  | $\text{H}-\overset{\text{O}}{\text{C}}-\overset{\text{CH}_3}{\text{CH}_2}-\overset{\text{CH}_3}{\text{CH}}-\text{S}-\text{CH}_2\text{CH}_2-\overset{\text{O}}{\text{C}}-\text{H}$ | $\text{Bis(1-Formylisopropyl) sulfide.}$                                                                  | 0.01-0.06                                |
| (c).....  | $\text{CH}_3\text{CH}_2\text{CH}_2-\text{S}-\text{CH}_2\text{CH}_2-\overset{\text{O}}{\text{C}}-\text{H}$                                                                         | 2-Formylethyl propyl sulfide.                                                                             | 0.0075-0.01                              |
| 6.....    | $\text{HO}-\text{CH}_2\text{CH}_2-\text{S}-\text{CH}_2\text{CH}_2-\text{SO}_2-\text{CH}_2\text{CH}_2-\text{S}-\text{CH}_2\text{CH}_2-\text{OH}$                                   | $\text{Bis(2-hydroxyethylmercaptoethyl) sulfone.}$                                                        | 0.005-0.015                              |
| 6(a)..... | $\text{HOCH}_2\text{CH}_2-\text{S}-\text{CH}_2\text{CH}_2-\overset{\text{O}}{\text{C}}-\text{OCH}_3$                                                                              | Methyl $\text{B}(2\text{-hydroxyethylmercapto) propionate.}$                                              | 0.004-0.0075                             |
| (b).....  | $\text{CH}_3\text{O}-\overset{\text{O}}{\text{C}}-(\text{CH}_2)_2-\text{S}-(\text{CH}_2)_2-\overset{\text{O}}{\text{C}}-\text{OCH}_3$                                             | Methyl $\text{B-Carboethoxyethylmercapto propionate.}$                                                    | 0.0075-0.015                             |
| 7.....    | $\text{HO}-\overset{\text{O}}{\text{C}}-\text{CH}_2\text{CH}_2-\text{S}-\text{CH}_2\text{CH}_2-\overset{\text{O}}{\text{C}}-\text{OH}$                                            | $\text{B},\text{B}'\text{-Thiodipropionic Acid.}$                                                         | 0.0075-0.03                              |
| 8(a)..... |                                                                                                 | Propyl-2-(a-pyridyl) ethyl sulfide.                                                                       | 0.005-0.01                               |
| (b).....  |                                                                                                | $\text{Bis}[2\text{-}(a\text{-pyridyl})\text{ethyl}] \text{ sulfide.}$                                    | 0.0075-0.015                             |
| 9(a)..... |                                                                                                | Methyl propyl $\text{B}[2\text{-N-methylpyridyl}-\text{ethyl}] \text{ sulfonium bis(methylsulfate).}$     | 0.005-0.01                               |
| (b).....  |                                                                                                | Methyl bis( $\text{B}-[2\text{-}(N\text{-methylpyridyl})\text{-ethyl}]$ ) sulfonium tris (methylsulfate). | 0.01-0.015                               |
| 10.....   |                                                                                                | Methyl $\text{B-methoxyethyl B-carbomethoxyethyl-sulfonium methylsulfate.}$                               | 0.01-0.015                               |

The second addition agent, which cooperates with the brightener in bright, acid, nickel plating solutions falls into the category of organic sulfonamides, sulfimides, and sulfonates.

The amount of control agent dissolved in the acid nickel plating solution ranges from .05 gram per liter to 20 grams per liter, best results being obtained from about 2 to about 5 grams per liter. These may be used in admixture as well as singly. That is, two control agents may be used instead of one, their combined concentration being kept within the above indicated limits.

It is to be understood that in the case of the sulfonamides, the radical corresponding to  $\text{X}$  in the general formula on page 1 may be written as carrying a negative

charge while the remainder of the compound may be written as carrying a positive charge, thus



or as written in column 1, lines 38 and 39.

TABLE II

## Aromatic sulfonamides

benzene monosulfonamide



saccharine, sodium salt



Table II—Continued

|                                                              |                                                                                                                                               |
|--------------------------------------------------------------|-----------------------------------------------------------------------------------------------------------------------------------------------|
| p-toluenesulfonamide                                         | $\text{CH}_3\text{C}_6\text{H}_4\text{SO}_2\text{NH}_2$                                                                                       |
| trichlorodibenzenesulfonamide                                | $\text{Cl}_2\text{C}_6\text{H}_3\text{SO}_2\text{NHSO}_2\text{C}_6\text{H}_4\text{Cl}$                                                        |
| di- $\beta$ -naphthalenesulfonamide                          | $\text{C}_{10}\text{H}_7\text{SO}_2\text{NHSO}_2\text{C}_{10}\text{H}_7$                                                                      |
| 4-carboxy dibenzenesulfonamide                               | $\text{C}_6\text{H}_5\text{SO}_2\text{NHSO}_2\text{C}_6\text{H}_4\text{COOH}$                                                                 |
| N,N'-bis(phenylsulfonyl)4,4'-diphenyldisulfonamide           | $\text{C}_6\text{H}_5\text{SO}_2\text{NHSO}_2\text{C}_6\text{H}_4\text{C}_6\text{H}_4\text{SO}_2\text{NHSO}_2\text{C}_6\text{H}_5$            |
| p,p'-oxy-bis(dibenzenesulfonamide)                           | $\text{C}_6\text{H}_5\text{SO}_2\text{NHSO}_2\text{C}_6\text{H}_4\text{OC}_6\text{H}_4\text{SO}_2\text{NHSO}_2\text{C}_6\text{H}_5$           |
| p,p'-methylene-bis(dibenzenesulfonamide)                     | $\text{C}_6\text{H}_5\text{SO}_2\text{NHSO}_2\text{C}_6\text{H}_4\text{CH}_2\text{C}_6\text{H}_4\text{SO}_2\text{NHSO}_2\text{C}_6\text{H}_5$ |
| <i>Aromatic sulfonates</i>                                   |                                                                                                                                               |
| benzene monosulfonic acid                                    | $\text{C}_6\text{H}_5\text{SO}_2\text{H}$                                                                                                     |
| benzene disulfonic acid                                      | $\text{C}_6\text{H}_4(\text{SO}_3\text{H})_2$                                                                                                 |
| nickel naphthalene disulfonate                               | $\text{C}_{10}\text{H}_6(\text{SO}_2\text{O})_2\text{Ni}$                                                                                     |
| cobalt naphthalene disulfonate                               | $(\text{C}_6\text{H}_5\text{SO}_3)_2\text{Co}$                                                                                                |
| nickel benzene monosulfonate                                 | $(\text{C}_6\text{H}_5\text{SO}_3)_2\text{Ni}$                                                                                                |
| dichlorobenzene disulfonic acid                              | $\text{Cl}_2\text{C}_6\text{H}_4(\text{SO}_3\text{H})_2$                                                                                      |
| toluene sulfonic acid                                        | $\text{CH}_3\text{C}_6\text{H}_4\text{SO}_2\text{H}$                                                                                          |
| diphenyl sulfonic acid                                       | $\text{C}_6\text{H}_5\text{C}_6\text{H}_4\text{SO}_3\text{H}$                                                                                 |
| thiophene sulfonic acid                                      | $\text{C}_4\text{H}_3\text{S}(\text{SO}_3\text{H})_2$                                                                                         |
| diphenyl sulfone                                             | $\text{C}_6\text{H}_5\text{SO}_2\text{C}_6\text{H}_5$                                                                                         |
| naphthalene trisulfonic acid                                 | $\text{C}_{10}\text{H}_5(\text{SO}_2\text{OH})_3$                                                                                             |
| <i>Unsaturated aliphatic sulfonamides and sulfonic acids</i> |                                                                                                                                               |
| sodium vinyl sulfonate                                       | $\text{H}_2\text{C}=\text{CHSO}_3\text{Na}$                                                                                                   |
| sodium allyl sulfonate                                       | $\text{H}_2\text{C}=\text{CHCH}_2\text{SO}_3\text{Na}$                                                                                        |
| vinyl sulfonamide                                            | $\text{H}_2\text{C}=\text{CHSO}_2\text{NH}_2$                                                                                                 |
| allyl sulfonamide                                            | $\text{H}_2\text{C}=\text{CHCH}_2\text{SO}_2\text{NH}_2$                                                                                      |

The constituents of the plating bath, according to the preferred practice of the invention, are (1) water, (2) nickel sulfate, nickel chloride, or a mixture of nickel sulfate and nickel chloride, (3) the brightener, (4) a sulfonate, a sulfonamide, a sulfimide, or one or more sulfonates, sulfonamides, sulfimides or mixtures thereof of the type previously indicated, (5) and a wetting agent (optional). An additional ingredient of the solution which is desirable is a buffering agent such as boric acid, formic acid, or the like.

It will be noted that in reference to the major constituent of the nickel plating solution, the solutions are similar to the well known "all chloride," "all sulfate," and "sulfate-chloride" or "Watts" type acid nickel plating solutions. The essential novel feature of the invention is the use of an acid nickel plating solution having one or more nickel electrolytes selected from nickel sulfate and nickel chloride and additionally containing cooperating

brightening agents, one of which is at least one carrier selected from the group consisting of unsaturated aliphatic sulfonamides, unsaturated aliphatic sulfimides, unsaturated aliphatic sulfonates, aromatic sulfonamides, aromatic sulfimides and aromatic sulfonates, and the other of which is a small amount of a brightener of the type heretofore indicated.

The basic solutions in connection with which the bright ductile nickel deposits are realized when containing the cooperating addition agents dissolved therein are as follows:

| ALL SULFATE                                  |                                                |  |
|----------------------------------------------|------------------------------------------------|--|
| 15 $\text{NISO}_4 \cdot 7\text{H}_2\text{O}$ | 100 to 400 grams, preferably 200 to 300 grams. |  |
| Boric acid                                   | 0 to 60 grams, preferably 10 to 40 grams.      |  |
| Wetting agent (e.g. sodium lauryl sulfate)   | 0 to 0.5 gram, preferably 0.05 to 0.2 gram.    |  |
| $\text{H}_2\text{O}$ to make 1000 cc.        |                                                |  |
| ALL CHLORIDE                                 |                                                |  |
| 20 $\text{NiCl}_2 \cdot 6\text{H}_2\text{O}$ | 50 to 250 grams, preferably 100 to 200 grams.  |  |
| Boric acid                                   | 0 to 60 grams, preferably 10 to 40 grams.      |  |
| Wetting agent (e.g. sodium lauryl sulfate)   | 0 to 0.5 gram, preferably 0.05 to 0.2 gram.    |  |
| 25 $\text{H}_2\text{O}$ to make 1000 cc.     |                                                |  |
| SULFATE-CHLORIDE WATTS TYPE                  |                                                |  |
| 30 $\text{NISO}_4 \cdot 7\text{H}_2\text{O}$ | 100 to 400 grams, preferably 200 to 300 grams. |  |
| $\text{NiCl}_2 \cdot 6\text{H}_2\text{O}$    | 10 to 60 grams, preferably 25 to 40 grams.     |  |
| Boric acid                                   | 0 to 50 grams, preferably 15 to 40 grams.      |  |
| Wetting agent (e.g. sodium lauryl sulfate)   | 0 to 0.5 gram, preferably 0.025 to 0.2 gram.   |  |
| $\text{H}_2\text{O}$ to make 1000 cc.        |                                                |  |

The plating solutions above identified may be operated under conditions of pH, temperature, and cathode current density which are customarily employed therewith. When the cooperating brightening agents of the invention are dissolved in the plating solutions in the amount previously indicated, bright, ductile deposits will be obtained upon electrolysis of the solution. Typical operating conditions for the basic solutions are as follows:

|                                                  | All Sulfate | All Chloride | Watts   |
|--------------------------------------------------|-------------|--------------|---------|
| 45 pH                                            | 3-4.5       | 2.4-4.5      | 3-4.5   |
| Temperature ° F                                  | 120-160     | 100-150      | 110-165 |
| Cathode Current Density (amp./ft. <sup>2</sup> ) | 20-40       | 60-200       | 30-70   |

In the preparation of the plating solution according to the invention, I add to each of the foregoing basic solutions a suitable quantity of the brightener and also one or more of the unsaturated aliphatic, or aromatic sulfonamides, sulfimides, and sulfonates. The plating solution for the best results, contains an antipitting agent although the deposits may be suitable for some purposes without eliminating pitting. Sodium lauryl sulfate or other wetting agents such as the sodium sulfate derivative of 7-ethyl-2-methyl-undecanol-4 and the dihexyl ester of sodium sulfosuccinic acid may be used as an antipitting agent, although its use is not essential and other wetting agents or mixtures of wetting agents may be used to control the pitting. For some purposes pitting may be tolerated and sometimes very little pitting occurs.

Specific examples of electroplating solutions containing different cooperating brighteners and carriers are illustrated in the following table which has been designated as Table III. It should be understood that the specific electroplating solution may be employed with or without air agitation. The operating conditions for obtaining bright ductile nickel deposits are also set forth in the table. In each case a bright nickel deposit of from 0.05 to about 1 mil thick or thicker, may be secured by electrolyzing the electroplating solution between an anode and a buffed brass cathode. Similar results may be secured on other types of cathodes conventionally employed

in acid nickel plating processes utilizing solutions of the type indicated herein.

TABLE III

|                                                                                 | Grams per liter |       |      |      |
|---------------------------------------------------------------------------------|-----------------|-------|------|------|
|                                                                                 | 300             | 300   | 300  | 300  |
| $\text{NiSO}_4 \cdot 7\text{H}_2\text{O}$                                       | 300             | 300   | 300  | 300  |
| $\text{NiCl}_2 \cdot 6\text{H}_2\text{O}$                                       | 40              | 40    | 40   | 40   |
| $\text{H}_3\text{BO}_3$                                                         | 40              | 40    | 40   | 40   |
| Sodium lauryl sulfate                                                           | 0.15            | 0.15  | 0.15 | 0.15 |
| Bis(2-hydroxyethyl) sulfide                                                     | 0.005           |       |      |      |
| Methyl B-(2-hydroxyethylmercapto) propionate                                    |                 | 0.005 |      |      |
| Methyl B-carbomethoxyethyl mercapto propionate                                  |                 |       | 0.01 | 0.01 |
| Propyl-2-( <i>o</i> -pyridyl)ethyl sulfide                                      | 3               | 3     | 3    | 3    |
| $[\text{C}_6\text{H}_5\text{SO}_2\text{NHHSO}_2\text{C}_6\text{H}_5]_2\text{O}$ |                 |       |      |      |
| Current Density, ASF                                                            | 40              | 40    | 40   | 40   |
| Temperature Range, °F                                                           | 140             | 140   | 140  | 140  |
| pH range                                                                        | 3.5             | 3.5   | 3.5  | 3.5  |

What I claim is:

1. An aqueous acid nickel plating solution comprising a source of nickel ions selected from the class consisting of nickel sulfate, nickel chloride and mixtures thereof, said solution also containing cooperating additives for enhancing the brightness of nickel deposits produced therein, one of said additives being chosen from the class consisting of aromatic sulfonates, aromatic sulfonamides, aromatic sulfimides, aliphatic sulfonates and sulfonic acids and the second being chosen from the class of compounds having the formula  $R-(\text{CH}_2)_n-S(\text{CH}_2)_n-R'$ , where  $n$  is an integer from 1 to 6,  $n'$  is an integer from 1 to 6,  $R$  is a member selected from the group consisting of



where  $m$  is an integer from 1 to 6,



where  $W$  is a hydrocarbon radical,  $X$  is an acidic radical selected from the group consisting of sulfate, sulfonate, halide and perchlorate radicals, and  $t$  is an integer from 0 to 1 inclusive, where  $R''$  and  $R'''$  are independently selected from the group consisting of hydrocarbon radicals and hydrogen;  $R'$  is a member selected from the group consisting of



where  $m$  is an integer from 1 to 6,



where  $R''$  and  $R'''$  are independently selected from the group consisting of hydrocarbon radicals and hydrogen wherein said second mentioned additive is present in solution in concentrations of from 0.0025 to 0.075 gram per liter, and said first mentioned additive being present in solution in concentrations of from 0.05 to 20 grams per liter.

2. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula

5 phatic sulfonamides and sulfonic acids, and the other of said cooperating additives being a compound of the formula



and being dissolved in said solution in concentration from 0.0025 to 0.075 gram per liter.

10 3. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



and being dissolved in said solution in concentration from 0.0025 to 0.075 gram per liter.

20 4. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula  $[\text{CH}_3-\text{O}-\text{CH}_2-\text{CH}_2]_n\text{S}$  and being dissolved in said solution in concentration from 0.0025 to 0.075 gram per liter.

25 5. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



30 45 an being dissolved in said solution in concentration from 0.0025 to 0.075 gram per liter.

50 6. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



55 60 and being dissolved in said solution in concentration from 0.0025 to 0.075 gram per liter.

65 7. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



and being dissolved in said solution in concentration from 0.0025 to 0.075 gram per liter.

8. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



and being dissolved in said solution in concentration from 0.0025 to 0.075 gram per liter.

9. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



and being dissolved in said solution in concentration from 0.0025 to 0.075 gram per liter.

10. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula



and being dissolved in said solution in concentration from 0.0025 to 0.075 gram per liter.

11. An aqueous, acid, nickel plating solution comprising nickel sulfate and nickel chloride and cooperating additives, one of said additives being present in solution in concentrations of from 0.05 to 20 grams per liter, and being chosen from the class consisting of aromatic sulfonates, aromatic sulfonamides, aromatic sulfimides, aliphatic sulfonamides and sulfonic acids, and the other of said cooperating additives being a compound of the formula  $\text{HOCH}_2\text{CH}_2\text{SCH}_2\text{CH}_2\text{SO}_2\text{CH}_2\text{CH}_2\text{SCH}_2\text{CH}_2\text{OH}$  and being dissolved in said solution in concentration from 0.0025 to 0.075 gram per liter.

12. An aqueous, acid, nickel plating solution comprising a source of nickel ions selected from the class consisting of nickel sulfate, nickel chloride and mixtures thereof,

said solution also containing cooperating additives for enhancing the brightness of nickel deposits produced therein, one of said additives being chosen from the class consisting of aromatic sulfonates, aromatic sulfonamides, aromatic sulfimides, aliphatic sulfonamides, and sulfonic acids and the second being chosen from the class of compounds having the formula



10 wherein  $n$  is an integer from 1 to 6,  $n'$  is an integer from 1 to 6,  $\text{R}$  is a member selected from the group consisting of



15 where  $m$  is an integer from 1 to 6,



30 where  $\text{R}''$  and  $\text{R}'''$  are independently selected from the group consisting of hydrocarbon radicals and hydrogen;  $\text{R}'$  is a member selected from the group consisting of



35 where  $m$  is an integer from 1 to 6,



where  $\text{R}''$  and  $\text{R}'''$  are independently selected from the group consisting of hydrocarbon radicals and hydrogen;

50  $\text{W}$  is a hydrocarbon radical;  $\text{X}$  is an acidic radical selected from the group consisting of sulfate, sulfonate, halide and perchlorate radicals and  $t$  is an integer from 0 to 1 inclusive wherein said second mentioned additive is present in solution in concentrations of from 0.0025 to 0.075 gram per liter, and said first mentioned additive being present in solution in concentrations of from 0.05 to 20 grams per liter.

60 **References Cited in the file of this patent**

**UNITED STATES PATENTS**

2,830,014 Gundel et al. \_\_\_\_\_ Apr. 8, 1958  
2,910,413 Strauss et al. \_\_\_\_\_ Oct. 27, 1959

UNITED STATES PATENT OFFICE  
CERTIFICATION OF CORRECTION

Patent No. 3,000,799

September 19, 1961

Jack L. Towle

It is hereby certified that error appears in the above numbered patent requiring correction and that the said Letters Patent should read as corrected below.

Column 1, lines 47 to 54, the third formula should appear as shown below instead of as in the patent:



column 2, line 50, for "a n" read -- an --; column 4, line 57, after "perchlorate" insert -- radicals --; columns 5 and 6, Table I-Continued, column 4, line 14 thereof, for "0.01-0.015" read -- 0.01-0.02 --; column 7, line 31, for "benzene" read -- benzene --; line 33, for "dichlorobenzene" read -- dichlorobenzene --; column 12, lines 8 and 9, the formula should appear as shown below instead of as in the patent:



Signed and sealed this 27th day of March 1962.

(SEAL)

Attest:

ERNEST W. SWIDER  
Attesting Officer

DAVID L. LADD  
Commissioner of Patents

Attest: